

Dec. 17, 1940.

A. D. MERRILL

2,224,976

# PROCESS AND APPARATUS FOR DIGESTING FIBROUS MATERIAL

Filed June 26, 1935



Inventor  
*ALBERT D. MERRILL*

Raymond J. Norton  
Attorney

## UNITED STATES PATENT OFFICE

2,224,976

PROCESS AND APPARATUS FOR DIGESTING  
FIBROUS MATERIAL

Albert D. Merrill, Watertown, N. Y.

Application June 26, 1935, Serial No. 28,578

5 Claims. (Cl. 92—7)

This invention relates to an improved process of and apparatus for digesting fibrous material, and more particularly to a method of controlling the characteristics of the digestion liquor during 5 the treating period.

As is known, in the preparation of sulphite pulp, the ultimate reaction involves an interaction between the lignin or its derivatives and the liquor. It is probable, or at least generally 10 assumed, that the bisulphite chemically combines with the lignin to form ligno-sulphonic derivatives, the action being generally conceived as a hydrolytic scission of the cellulose-lignin aggregates or esters. Coincidentally a number 15 of more or less complicated secondary hydrolytic reactions occur, resulting in the formation of such products as sugars, variant forms of hydrolyzed cellulose and the like. Usually a base, such as calcium or magnesium, is employed upon the 20 theory that these combine with certain products of hydrolysis and prevent further reaction of such products. It is generally assumed that the reactions, *inter alia*, include the formation of organic acids which then combine with the sulphites to displace and set free an equivalent amount of sulphurous acid, this liberation being greatest in the latter part of the cook and necessitating a blow down to diminish the pressure. 25

Whatever may be the precise mechanism of 30 the reaction, it is a practical fact that the concentration of the sulphurous acid is the most important factor, considered not only as a component of the reagent, *i. e.* in chemical combination with the base, but also in the free or uncombined state.

This importance has of course been recognized and many suggestions have been advanced as to 35 methods of maintaining the acid concentration during the reactions. Of these perhaps the one of most practical importance and value is the recirculation of the free gas back into the body of the digestion liquor. The usual method of accomplishing this is to couple a gas line and a liquor line into the same circuit and to withdraw 40 and readmit both gas and liquor by means of a pump. Ramifications of such a method include 45 the suggestion of effectively condensing and/or absorbing the gas during this passage, as by means of a jet condenser or eductor.

The present invention relates to this general 50 type of treatment, that is to a method of maintaining acid concentrations by returning free gas either continuously or intermittently to the body of the liquor in the digestion zone. In common

with prior art suggestions also the present invention utilizes a recirculating stream of liquor as the carrier and absorber of such gas. The present method however is fundamentally different from those heretofore employed principally in that it 5 involves the selective recirculation of gas and liquor. By reason of this the chemical characteristics of the cooking liquor may be accurately controlled and, if desired, optionally varied during the progress of the cook to thus obtain an 10 improved result. Other concomitant advantages obtain which will be described hereinafter or which will clearly appear from a consideration of the novel method.

An object of the present invention therefore is 15 to provide an improved process of digesting fibrous materials.

Another object is to provide a new method of handling or manipulating a digestion liquor 20 which includes as one of its components a relatively volatile gas.

Another object is to provide an improved type 25 of gas-liquor circuit for use in the digestion of fibrous materials.

A further object is to provide a novel method 30 of controlling the chemical characteristics of a digestion liquor during the treatment of fibrous materials.

With these and other equally important objects 35 in view, the invention comprehends the concept of digesting fibrous material with a digestion liquor, one component of which is a volatile material, such as sulphur dioxide, and selectively recycling the liquor and gaseous component during 40 the treatment.

In order to enable a more ready comprehension 45 of the underlying principles of the present invention, a typical arrangement of apparatus by which it may be effectuated is shown in the single figure of the accompanying drawing, the purpose being to illustrate the fundamental mode of operation rather than to exclusively define the apparatus which is available. For this reason and further to simplify the drawing, conventional 40 units have been selected.

As indicated hereinbefore, it has been suggested 50 prior to this time to withdraw evolved gases from the upper portion of a digester and introduce them into a recirculating stream of digester liquor. In such prior methods the gas and liquor lines were connected in the same circuit, usually through an eductor, and the amount of gas which was withdrawn in any given time was dependent upon or a function of the velocity of 55

the liquid stream. Thus it was substantially impossible to control the flow of the gas independently of the flow of liquor or to maintain any desired gas pressure independently of the recycle stream except by blowing off through a relief, in which case potential control of concentration was lost to the extent of the amount of gas removed from the circuit.

The present invention on the other hand, as 10 intimated, involves the independent or selective control of the amount of recycled gas as compared to the amount of recycled liquor. In this way, therefore, control of the concentration of the acid by means of optionally varying the 15 partial pressure of the sulphur dioxide gas in the vapor space may be obtained without necessarily recycling an equivalent quantity of liquor. Thus, utilizing the principles of the present invention, a substantially constant flow of liquor may be 20 established in the recycle circuit, and the flow of gas may be varied independently of the liquor to adjust the concentration at any desired stage of the cook. Furthermore, in the improved embodiment of the invention the gas recycle line, 25 due to this fact of independent control, may be utilized for other purposes, such for example as rapidly relieving gases during the latter stage of the cook or for withdrawing excess gases from the digestion zone for transportation to some 30 other absorption system. These and other advantages may be achieved in operating a process which may be carried out in the apparatus shown.

In the drawing 1 indicates an acid storage 35 tank of any suitable size and construction. This, as is known, may be supplied with fresh acid from the acid towers by means of the supply line 2 and pump 3. Liquor may be taken from storage tank 1 by the pump 4 and forced through line 5, check valve 6 and eductor 7 to the drop 40 leg 8. This drop leg is connected at its lower end with the second eductor 9 and thence through the branch 10 to the accumulator 11. The eductors are provided with control valves 7' and 9' respectively, the purpose and operation of which 45 is described in prior Patent 1,888,632.

With such an assemblage it will be appreciated that relatively cool acid may be pumped from the acid storage through eductor 7, drop leg 8 and eductor 9 into the accumulator and 50 that during such passage acid may be employed to absorb gas and condense condensable vapors.

As described more fully in Patent 1,918,459, the absorption or condensation of gases and vapors may be accentuated by associating the 55 eductor 9 with an accumulator recirculation circuit. As shown, this may comprise the inlet branch 12, controlled by valve 12', pump 13 and branch line 14, which latter communicates with the liquid inlet of eductor 9. With this type of 60 circuit liquor may be withdrawn and forced by the pump 13 at any desired velocity through branch 14 and into eductor 9, and thence to the accumulator through the branch 10. Liquor flowing through line 14 absorbs and condenses 65 gas and/or vapors flowing downwardly through the drop leg 8 in admixture with liquor.

The temperature of the acid within the accumulator may be more accurately controlled by 70 interposing, if desired, a heater in this recirculation line, as fully described in Patent 1,918,459.

The pressure within the accumulator may likewise be controlled. As shown, a vent line 15 leads from the upper or vapor section of the spherical accumulator and is immersed to a considerable depth in the liquor contained in acid

storage tank 1. In this line is interposed the pressure regulating valve 15'. This may be set at any desired value of the order of 30 lbs. more or less so that when the pressure in the accumulator exceeds this setting, gases are automatically vented through line 15 and are absorbed within the acid within the storage tank. 5

The digestion of the material is carried out in one or more digesters 16. These may be of typical or conventional construction and include the 10 removable manhole cover 17 and a valve blow off elbow. Each one of the digesters is provided with a gauge glass 18, for the purpose of determining the liquor level, and pressure indicating or recording instruments (not shown). The relief line 20, having the interposed control valve 20', connects with the main or high pressure header 21. Similarly the side relief 22, having control valve 22', communicates with header 21. This latter, as shown, leads to the eductor 7. 20 Fluids may flow from the digester through either or both lines 20 and 22 into header 21 and thence in the manner described through the drop leg 8 into the accumulator. Such hot fluids precondition and preheat the cooler acid flowing through 25 line 5.

The digester is also provided with a low pressure relief line 23, having a control valve 23', and is connected to the header 24. This latter header, which carries the low pressure gases, terminates 30 below the liquid level in the acid storage. The digesters are also provided with the air vent branches 25, controlled by valve 25', through which displaced air may be vented during filling 35 of the digester, in a manner to be particularly described.

The lower end of the digester is connected, by suitable branch lines 26, to a steam header (not shown) in the usual manner. A bypass line 27 provided with a pressure regulating valve 27' 40 may extend from the header 21 to the accumulator 11. This line serves automatically to bypass fluids around the eductor to the accumulator when the pressure in the latter drops to a predetermined degree. 45

The top, side relief and bypass lines described above are now well known in the art and are described fully in U. S. Patent to Dunbar 1,918,459.

The digestion liquor, for the purpose either of 50 preheating the acid prior to cooking or for directly cooking the material in the digester, may be fed from the accumulator 11 through line 30, controlled by valve 30', and pump 32, into the feed header 33. From this header the hot pre-conditioned acid may be admitted to the several 55 digesters through the branches 34, controlled by valves 34'.

By opening valve 30' and valve 34' on a particular digester, hot acid may be forced by means of the pump (supplemented by the existing pressure in the accumulator) into the bottom of the digester until such digester is filled under any desired hydrostatic pressure. After filling the 60 digester may be sealed off from the supply in accumulator 11 by manipulating valve 34'. 65

In a process of the present type it is desirable to recirculate both gas and liquor to and from the digester. For this purpose the recirculation circuits of the type shown are employed. As 70 will be observed from an inspection of the drawing, liquor may be withdrawn from the upper portion of the digester through the line 40 by means of the pump 41 and then forced through line 42, heat control unit 43 and eductor 44 to the digester. If desired the eductor 44 may be 75

cut out of this circuit and the recycle liquor passed through line 45, having a control valve 45'.

While the liquor recycle circuit is shown as one involving the withdrawal of liquor from the upper and returning it to the lower portion of the digester, it will readily be appreciated that by the proper placement of the lines or by the use of proper branch and bypass connections, the circulation may be in the opposite sense, namely 10 from the bottom to the upper portion. It is further to be understood that the invention comprehends the utilization of these two circulations, namely top to bottom and bottom to top, during any given treatment. Since the method of 15 achieving this is well known to those skilled in the art and since a showing would unduly complicate the drawing, such reverse circuits are not shown.

Consonant with the principles of the invention 20 as described hereinbefore, means are provided to withdraw gas from the upper or gas space of the digester and force it by independent means into the bottom of the digester. Preferably, since a liquid recycle circuit is being employed, the 25 two are combined in such a way as to absorb the gases and condense vapors passing through the gas line, and for this purpose the eductor 44 is utilized.

Such separate gas recycle circuit may comprise 30 the line 50, one end of which is positioned within the vapor space of the digester. The end of this line is suitably screened in the manner well known in the art. The other end of the line 50 is connected to the intake of a compressor or 35 blower 51, such as a Roots blower or a Nash blower. The outlet of the blower is connected through line 52 which may discharge directly, as shown, into the digester. Connected to the line 40 52 are a number of branch lines through which the gas may be caused to flow. Thus gas withdrawn from the upper portion of the digester may be forced through branch 53, which branch is controlled by valve 53'. This branch connects with the discharge or high pressure side of pump 41 45 and such points of connection may be made either anterior or posterior to the heater 43.

If desired the discharge of the pump and branch 53 may connect with an enlarged chamber to provide a greater area for the mixing of 50 the gas and liquid. To facilitate such mixing agitating means may be provided within the container. In any event it will be observed that in such circumstances gas and liquid may separately and independently be withdrawn from the 55 upper portion of the digester and admixed and combined in a zone of high hydrostatic pressure, thus insuring a greater absorption of gas and condensation of condensable components. Either before or after such admixture the fluids may be 60 passed through the heater so as to raise the temperature to any desired value.

Likewise if desired, the branch 53 may be cut out by closing the valve 53' and the gas forced 65 through line 52 and branch 54 into eductor 44. The flow of the gas through this branch may be controlled by valve 54'. Wherever the circumstances require both branches 53 and 54 may be cut out and valve 55' opened so as to pass the gas through lines 52 and 55 into the bottom of the 70 digester.

Similarly it will be understood that if and when desired valve 55' may be closed and both valves 53' and 54' opened so that gases from line 52 flow into the branch 42 and into the liquid line through the eductor. When either line 53

or 54 is opened and operating it will be appreciated that the suction created in these lines supplements the action of the blower 51 in rapidly flowing the gas through the recycle line.

As noted hereinbefore the separate gas recycle 5 line may be employed for additional purposes during the course of treatment. Thus valves 53', 54' and 55' may be closed and gases may be withdrawn from the upper portion of the digester and caused to flow through the valve branch line 56 10 for suitable disposition. Thus for example line 56 may be connected to the accumulator 11 or by suitable conduits to another digester for the purpose of increasing the free acid content and adding heat units to the liquor in such digester. 15 Again a branch from line 56 may lead to a low pressure accumulator or storage tank so that gases vented during the filling of the digester may be absorbed in such tank. By utilizing a blower in this line the final blown down period 20 may be materially shortened inasmuch as the pressure can be rapidly relieved by the blower rather than by the slower method employed heretofore.

Also it will be observed that the separate gas 25 line may be used together with the liquid recycle line at or near the end of the cook for the purpose of degassing the liquor. In these circumstances liquor may be withdrawn from the bottom portion 30 of the digester, in a manner heretofore described, and pumped to the top of the digester to be sprayed therein. By operating the blower 51 at this time the pressure in the vapor space may be materially diminished and the free gas quickly 35 evolved from the liquor and withdrawn through lines 52 and 56 for utilization elsewhere in the system. It is to be observed that in these circumstances degassing is very rapid because the blower 51 tends to establish a reduced pressure in the vapor space of the digester and thus accelerate the evolution of gas from the recycle liquor which is sprayed into the top. Such method therefore insures not only economies in operating time but maximum recovery of chemical values.

It will be appreciated that inasmuch as the 45 centrifugal pump 41 and the blower or equivalent motive power 51 are independently operated, the flow of the respective materials, namely the gas and liquor, may be varied to any desired degree and at any time. In this manner, therefore, it 50 is possible to insure a rapid recirculation of gas and a relatively slower recirculation of liquid. This is in sharp contradistinction to prior art proposals in which the flow of gas was of necessity a function of the flow of recycled liquor. This 55 type of procedure therefore establishes a method of controlling the partial pressure of the gas in the vapor space which could not be achieved heretofore. The degree of this control can of course be modified over a relatively wide range. Thus, 60 if desired, there may be connected into the gas recycle line a separate source of gas, that is to say gas from an extraneous source may be admitted to the gas recycle line and thus caused to enter the gas recycle circuit to increase the partial pressure of 65 the SO<sub>2</sub> in the digestion zone. This may readily be done by connecting to the gas recycle line a tank of gaseous or liquid SO<sub>2</sub>. As noted hereinbefore, by opening the branch line 56 to the desired degree gas may be withdrawn from the circuit to 70 any desired extent and, as explained, towards the end of the process may be used, in conjunction with the liquid recycle line, to substantially completely evacuate the circuit of free gas.

In addition to these major advantages by rea- 75

son of which the chemical characteristics of the process may be controlled, it will be observed that the particular arrangements provide so-to-speak mechanical advantages. For example, by utilizing the separate blower for the gas and the centrifugal pump for the liquid, the fluids may be combined as described in a high pressure zone, on the discharge side of pump 41, thus insuring the same effective operation of both the pump and the blower and an optimum absorption of gas. By utilizing such an arrangement and by placing the liquor inlet 40 well below the normal liquid level in the digester, it will be appreciated that all difficulties of gas binding of the centrifugal pump are avoided.

The complete process for producing pulp from ligno-cellulosic material will have been appreciated from the foregoing description. In carrying out such a process the raw material, such as wood chips, is admitted to the digester through the open manhole 17. After the digester has been completely filled with chips the cover is bolted on and valve 25' is opened, valves 20', 22' and 23' at this time being closed. Hot pre-conditioned liquor is then forced from accumulator 11, in the manner described, through branch 34, into the bottom of the digester. As the liquid level rises air is continuously displaced and is vented through the open valve 25'. When the air is completely vented and SO<sub>2</sub> gas begins to discharge at valve 25' the valve in line 50 may be opened and blower 51 operated to withdraw gases from the digester and pass them through line 56 to a branch line (not shown) into the acid storage tank. When such gases are withdrawn and the digester filled, the valve in line 50 may be closed and operation of the blower 51 discontinued. Then preferably the pump 30 is continued in operation until a high hydrostatic pressure is built up upon the liquid. This pressure (gauge) may, for example, vary from 40 to 300 lbs. or more per sq. in. The chips are then in contact with liquid under high pressure and at an elevated temperature but below reaction temperatures, the temperature of the acid withdrawn from the accumulator 11 being normally at about 70 to 110° C.

After the high hydrostatic pressure has been built up on the acid, valve 34' is closed and the liquid recirculated to and from the digester for a period of from one to six hours, so as to insure a thorough saturation of the chips with the liquor. During the saturation period no recirculation of gas is necessary. At this time however, if desired, gas may be admitted to the liquid recirculation line from an extraneous source so as to build up the partial pressure of the SO<sub>2</sub> in the digestion zone and thus increase the concentration of the acid during the saturation period without increasing the temperature. During the saturating period the temperature of the acid may be maintained at the optimum value by indirectly heating recycle liquid in the heater 43. In this manner the chips may be thoroughly saturated with hot acid at an optimum concentration and temperature. If the optimum saturating concentration is less than the concentration to be employed for cooking, sufficient gas can be withdrawn from the circuit to reduce the concentration to the desired value.

At the termination of the saturating period, which as noted above may vary over a considerable period of time, conditions within the digester are adjusted so as to bring the mass up to reaction temperatures. As shown in the

drawing, this may be done by opening valve 22' and relieving liquid from the digester to lower the liquid level to the desired point. At this time also, if desired, the blower 51 may be operated for a short period of time to withdraw gas from the zone and thus to adjust the concentration of free gas prior to cooking. Then the mass is brought to reaction temperature by applying heat, either by means of a closed steam coil or preferably as shown by introducing direct steam through the branches 26.

Sometime after the initial admission of steam the valve 20' may be opened, thus venting fluids to the desired extent from the digester to the header 21 and thence through the described circuit to the accumulator.

After a period of time, which may vary depending upon the particular conditions of the treatment, the valve 20' may be closed and the valve 22' in the side relief line opened to withdraw liquid and to maintain the liquid level at the desired point. The continued introduction of steam, by reason of condensation, increases the volume of liquid within the digester. This volume is indicated by the gauge glasses 18 and 25 such volume may be adjusted, in the manner well known to those skilled in the art, by proper manipulation of the relief valves.

Either continuously or intermittently during the cooking period liquor may be withdrawn from the upper portion of the digester, through line 40, and forced under the pressure of pump 41 into the lower portion. Contemporaneously gas may be withdrawn from the vapor space of the digester through line 50, under the action of blower 51, and then admixed with the liquid in a zone of high hydrostatic pressure, through line 53, or in the eductor through line 54, or finally whenever circumstances recommend, directly into the digester through line 55.

While the pump 41 has been shown as a centrifugal pump adapted, due to its operation, to force a steady stream of liquor through the circuit, it will be appreciated that this may be replaced with a reciprocating pump so as to introduce the liquor into the digester in a series of pulsating or surging streams, in the manner described for example in the prior application of T. L. Dunbar, Serial No. 636,312, filed October 5, 1932. This type of introduction of liquor provides the advantage of agitating or loosening up the body of the pulp. As noted above, during the cooking period liquor may be withdrawn from the bottom and admitted to the top of the digester and a combination of these two types of recirculation, namely from top to bottom and bottom to top, may be utilized.

With this type of operation the quantity of gas recycled at any particular time may be varied entirely independently of the quantity of liquor, and the gas and liquor may be combined under such conditions as to insure optimum absorption and heat control. By utilizing the gas recycle line, as noted hereinbefore, SO<sub>2</sub> gas (or its equivalent) may be introduced from an extraneous source to build up the partial pressure of the gas in the digestion zone, or any predetermined amount of gas may be bled from this line.

It will thus be appreciated that the concentration of the acid during any stage in the cook may quite accurately be controlled without modifying to any considerable degree the original concentration of the acid, that is to say the concentration of the acid at the start of the cook.

As the reactions involved in the digestion of

ligno-cellulose proceed, that is to say in the latter part of the cook, organic acids formed combine with sulphites present and tend to displace an equivalent amount of sulphurous acid. In order to maintain the proper pressure conditions the evolved gas should, as is known by those skilled in the art, be withdrawn. In the present process this may be done as in the past by bleeding off through line 23 or by withdrawing such gas from the gas recycle line through branch 56, or by a combination of both. It will be appreciated that in this stage of the cook the pressure within the digester may be more quickly or responsively controlled since the blower 51 may be operated to suck out these gases at a relatively more rapid rate than could be done heretofore through the low pressure line. It will also be appreciated that when the blower 51 is employed for withdrawing gases during this "blow off" stage of the cook, not only more rapid withdrawal may be achieved but a greater absorption of gas may be secured, for the outlet branch 56 may be connected to an absorption system in which a higher pressure obtains than in the acid storage tank.

After the termination of the cook and before the pulp is discharged from the digester, as indicated hereinbefore, maximum recovery of chemical values may be obtained by utilizing the dual recycle circuit. For this purpose the liquid in the digester, now under relatively low pressure, may be withdrawn from the bottom and forced to and sprayed into the top of the digester. At this time the blower 51 may be operated to set up a diminished pressure in the upper portion of the digester, thus increasing the evolution of SO<sub>2</sub> gas and withdrawing this from the digestion zone. Thus the residual or spent liquor may be denuded practically completely of its free gas by an improved type of operation which in fact comprises a rapid reduced pressure distillation.

If desired the liquid recycle line may be employed, by connecting it to suitable separate inlet lines, to force a washing solution through the pulp prior to discharge of the pulp to the pulp storage. After such discharge the pulp may be further processed in the manner well known to those in the art.

It will be observed, therefore, that the described system presents many advantages over those heretofore employed. The provision of a separately controlled gas recycle line enables a more accurate adjustment of pressure during any stage of the cook; it insures increased absorption of the free gas by enabling the utilization of a high pressure zone for the absorption, while at the same time it permits more efficient operation of the liquid pump. The use of this type of gas recirculation system, as pointed out, permits the possibility of employing it for a number of other and advantageous purposes or functions, such for example as rapid degassing of the residual liquor in the manner described. While, therefore, the novel gas-liquid recycle circuit has been described with respect to employment on a digester and during the cooking period, it will be appreciated

that the fundamental principles may be embodied in any step of the treatment in the plant.

Therefore, while preferred procedures and apparatus have been described, it will be understood that these are given as illustrative of the underlying salient principles of the invention and not as delineating the scope of the invention. 5

I claim:

1. In a process of digesting fibrous material, pumping acid liquor directly to and from a digester through an acid liquor circuit, separately pumping a stream of hot gas from the upper portion of the digester, and in an amount independent of the amount of liquor passing through the liquor circuit, admixing this with the stream of liquor in the high pressure section of the liquor circuit and introducing the admixed stream to the digester. 10

2. In a process of digesting fibrous material, pumping a stream of acid liquor through a circuit from one section to another section of the digester, during the cooking period, separately pumping a stream of gas from the upper portion of the digester and forcing it into the lower portion of the digester during the cooking period; 20 then during the latter stages of the treatment withdrawing liquor from the bottom and spraying it into the top of the digester, and utilizing said gas circuit to impose a reduced pressure on the digester to increase the evolution of gas from 25 the liquor and to withdraw evolved gas from the digester. 30

3. An apparatus for digesting fibrous material comprising a digester, a liquor recycle line extending from the upper to the lower portion of 35 the digester, a pump and heater and eductor in such line, a gas recycle line extending from the upper to the lower portion of the digester, a blower in such line, and means optionally to connect such gas line directly to such liquor line 40 on the pressure side of the pump or through said eductor. 40

4. An apparatus for digesting fibrous material comprising a digester, a liquid recycle line extending from the upper to the lower portion of 45 the digester, a pump and heater and eductor in such line, a gas recycle line extending from the upper to the lower portion of the digester, a blower in such line, and means to connect such gas line to such liquor line on the pressure side of 50 the pump. 50

5. In a process of digesting fibrous material, filling a digester with the material, admitting acid to the digester and simultaneously displacing air therefrom, continuing the admission of acid and withdrawing evolved gas through a line having an interposed blower and conducting such gases to a storage tank; subsequently digesting the material at superatmospheric pressure with the liquor while recycling liquor to and from the digester and separately recycling gas to and from the digester through a circuit including the blower and at a rate of flow independent of the rate of flow of liquor through the liquor circuit. 55 60

ALBERT D. MERRILL.